

1

2,971,827

## FUEL OIL ADDITIVE

Arthur V. Churchill, Oakmont, and Edward Mitchell, Valencia, Pa., assignors to Gulf Research & Development Company, Pittsburgh, Pa., a corporation of Delaware

No Drawing. Filed Dec. 2, 1957, Ser. No. 699,910

10 Claims. (Cl. 44—64)

This invention relates to improving the combustion characteristics of hydrocarbon oil fuels that normally tend to form substantial amounts of soot and smoke during combustion, and to improve agents adapted for use in such fuels.

The petroleum industry has encountered a serious problem in satisfying the demand for middle distillate and heavier fuel oils that can be burned in fuel burners such as those of the atomizing type and of the rotary wall flame type with little or no accompanying formation of smoke or soot. Oils that are normally burned in oil burners of the types indicated are those of Number 2 grade or heavier, although lighter oils can be used. Although some smoke and soot formation will normally accompany combustion of any suitable oil in burners of the type indicated, especially where less than optimum combustion conditions are used, the problem is serious in the case of oils having an API gravity of less than 34°, as substantial smoking and soot formation will occur during combustion of such oils even when favorable combustion conditions are employed. The poor combustion characteristics of such oils are considered attributable to the relatively high proportion of aromatic components contained therein. Fuel oils having an API gravity of less than 34° will normally contain in excess of about 20 percent aromatics, for example, 25, 40, or even 60 percent or more of aromatic components, whereas lighter fuel oils will normally contain a substantially lower proportion of aromatics, for example, 15 percent or less. In the case of distillate oils, a high aromatics content usually signifies a large proportion of cracked distillates, as the latter are relatively rich in aromatics. The proportion of catalytically cracked distillate fuel oils in commercially marketed fuel oils has increased in recent years notwithstanding the relatively inferior burning qualities of such oils, because the demand for fuel oils of comparable boiling range has exceeded the available supply of straight-run oils.

Not only do low-gravity distillate oils containing large proportions of cracked distillates, that is, oils rich in aromatics, form greater quantities of soot during combustion than straight-run, high-gravity distillate oils, or similar oils low in aromatics, but also such oils form soot of different quality. Soot formed from the latter oils is a loosely deposited, low-density material having a low coefficient of heat transfer, whereas soot from the former oils is resinous, much denser and has a higher coefficient of heat transfer.

While the problem of clean combustion is especially serious in the case of distillate fuels, where fuel quality is of major importance, a combustion problem also exists in the case of residual fuel oils. Similarly as the middle distillate fuel oils, the residual fuels have an API gravity less than 34° (API gravity for typical No. 6 fuel oils varies in the range of 5° to 15°), and they also fre-

2

quently contain exceptionally large proportions, for example 60 percent or more, of aromatic components. Residual fuels can contain relatively low-boiling aromatic components as well as higher boiling materials, as they are frequently diluted or cut-back with lower boiling cracked distillate oils in order to reduce the viscosity of the heavier oils.

Although the combustion of fuel oils having an API gravity of less than 34°, and consequently a relatively large proportion of aromatics, will tend to produce soot and smoke in various ordinary atomizing type burners, that is, burners in which the fuel oil is burned in the form of a spray of liquid droplets after mixture with air, combustion of such oils in rotary wall-flame type burners constitutes an especially severe problem. In the latter instance the fuel oil is burned in vapor form after vaporization of the fuel by impingement thereof on a hot metal surface.

Excessive smoking and soot formation during combustion of fuel oils is objectionable not only from the standpoint of cleanliness and air pollution, but also in that smoke and soot lead to stack deposits which may reduce burner draft and/or cause the stack temperature to rise to a dangerous point.

The present invention relates to improved fuel oil compositions comprising hydrocarbon fuel oils that have an API gravity of less than 34°, which compositions have reduced smoke and soot forming tendencies during combustion, whereby such fuel oil compositions are rendered more suitable for use as fuels in domestic oil burners of various kinds, such as heating furnaces of the atomizing or rotary wall-flame type, combustion gas turbine engines, diesel engines and the like. We have found that such improved fuel compositions can be obtained by incorporating in a fuel oil of the type described and that normally tends to form substantial smoke and soot during combustion, a small amount of a salt of an oil-soluble hydrocarbon sulfonic acid and hydrazine. For example, excellent results have been obtained with monohydrazinium polydodecylbenzene sulfonate. Specific examples of other suitable salts include dihydrazinium polydodecylbenzene sulfonate and mono- and di-salts of hydrazine and oil-soluble petroleum sulfonic acids. The invention includes fuel oils containing these salts as well as the salts themselves.

The exact mechanism by which the hydrazinium sulfonates disclosed herein function to reduce smoking and sooting during combustion of fuel oils of the class disclosed has not been definitely determined, and accordingly, we do not intend the present invention to be limited to any particular theory of operation. It may be that the hydrazinium sulfonates reduce the ignition temperature of the oil, thus enabling more complete combustion and at the same time reducing the possibility of thermal cracking of the oil prior to combustion. On the other hand, it may be that the hydrazinium sulfonates cause the oil to burn at a higher temperature, thus facilitating more complete combustion. Regardless of the mechanism by which the agents disclosed herein function, available experimental evidence shows that a definite reduction in smoke and soot forming tendencies is obtained by the use of small amounts of these agents in fuel oils that normally tend to promote excessive soot and smoke formation during combustion in atomizing type burners.

The hydrazinium sulfonates of this invention can be prepared in any convenient manner. For example, they can be prepared by direct reaction of hydrazine with the desired oil-soluble sulfonic acid in a mol proportion in

the range of about 1:1 to 1:2. The neutralization reaction takes place spontaneously at atmospheric conditions of temperature and pressure. However, other conditions can be used. For example, mild heating, say up to 160° F., can be resorted to provided the heat is insufficient to decompose the addition salt.

The nature of the acidic portion of the hydrazine salts is important insofar as the combustion-improving characteristics of the salts are concerned. Thus, salts of hydrazine and oil-soluble hydrocarbon sulfonic acids have been found to possess exceptional advantages from a combustion-improvement standpoint. For example, especially effective results have been obtained with salts of hydrazine and long-chain aliphatic hydrocarbon-substituted benzene sulfonic acids, particularly the monohydratium sulfonate, that is, the salt produced by reacting hydrazine and a long-chain aliphatic hydrocarbon substituted benzene sulfonic acid in approximately equimolar proportions. By "long-chain aliphatic hydrocarbon-substituted benzene sulfonic acid" is meant a benzene sulfonic acid having as a nuclear substituent a hydrocarbon chain of a length and configuration such as to impart fuel oil solubility to the acid. The long-chain aliphatic hydrocarbon groups can be saturated or unsaturated, straight or branched chain and/or substituted with substituents that contain elements or groups other than carbon and hydrogen and that do not interfere with oil-solubility or other fundamental characteristics of the ultimate salt, for example, oxygen, hydroxyl, carbonyl, amino, halogen, sulfur, mercapto and the like. Examples of oil-soluble, aliphatic hydrocarbon-substituted benzene sulfonic acids that possess sufficient fuel oil solubility to form suitable salts for the purposes of this invention include ortho and para tetradecyl, hexadecyl, octadecyl, triacontanyl and polydodecyl benzene sulfonic acids. The invention is not limited to long-chain aliphatic hydrocarbon-substituted benzene sulfonic acid salts, however, and salts of other oil-soluble hydrocarbon sulfonic acids can be used. Thus, oil-soluble petroleum sulfonic acids, that is, mahogany acids, can also be used to form mono- and dihydrazinium salts useful for the purposes of the present invention.

The hydrazinium sulfonates included by this invention are added to the fuel oils in a proportion sufficient substantially to reduce the smoking tendencies of the oil. Since the various materials disclosed herein are not necessarily exact equivalents, the optimum proportion will vary according to the nature of the particular agent added, and to some extent according to the nature of the fuel oil. The type of fuel oil burner employed can also affect the optimum proportion of agent to be added. Within the limits of these considerations, we have found that best results are obtained by addition to the fuel oils of small amounts of the hydrazinium sulfonates disclosed herein. Thus, noticeable improvement usually will be obtained by addition of as little as 0.02 weight percent of these materials to the fuel oils, and a major improvement will be obtained by the addition of about 0.05 weight percent to the fuel oil. Normally, it will not be necessary to add the hydrazinium sulfonates in excess of 0.2 weight percent of the composition, although in some cases it may be desirable to employ as much as 0.5 percent of the salt.

The compounds disclosed herein may be incorporated in the fuel oil in any suitable manner. Thus, the hydrazinium sulfonates can be added to the fuel oil either as such or in the form of concentrated mineral oil solutions. After addition of these materials to the oil, some circulation of the oil is desirable to facilitate early formation of a homogeneous composition, but this is not absolutely essential.

In order to demonstrate the effectiveness of the combustion improvement agents disclosed herein, hydrazine sulfonate was incorporated in a No. 2 fuel oil that normally tends to form smoke and soot on combustion, and

the thus-compounded fuel oil was tested for smoking tendencies by combustion in an atomizing type burner. The test was carried out in a domestic oil burner (Timken, Model OFH-60Hi-Furnace). Conventional burner controls were associated with the test apparatus in conjunction with electrical timer relays to provide a 20 minute on 10 minute off cycle of burner operation. After permitting a warm-up of at least one 20 minute on cycle of burner operation with maximum combustion air, smoke spot and CO<sub>2</sub> reading were taken at the middle of each on cycle for 7 cycles using different air gate settings to regulate the quantity of combustion air. Changes of gate setting were made during burner "off" phases of the cycle. Smoke spot readings were obtained by withdrawing flue gas from a sampling probe installed in the chimney pipe through a disc of No. 4 Whatman filter paper one inch in diameter for 2 minutes. A vacuum pump was used to maintain a pressure differential of 2 1/4 inches Hg across the disc. The smoke spot reading was then determined by means of a photocell meter which had been calibrated using a Shell smoke spot chart graduated in increasing shades of black ranging from zero (clean disc) to 9 (black disc) as the standard. The CO<sub>2</sub> readings were obtained by withdrawing flue gas through a sampling probe installed in the chimney pipe (according to United States Department of Commerce Bulletin CS104-46) and by analyzing the flue gas for percent CO<sub>2</sub> in an Orsat-type flue gas analyzer.

The test fuel, hereafter referred to as test fuel A, was an uninhibited commercial-type, 30° API gravity No. 2 fuel oil having an aromatics content of about 45 percent and consisting of 36.4 volume percent straight-run No. 2 fuel oil distillate and 63.6 volume percent catalytically cracked No. 2 fuel oil distillate.

Percentages given herein are by weight of the composition unless otherwise specified. The term "No. 2 fuel oil" is defined in "ASTM Standards on Petroleum Products and Lubricants for November 1956" as a distillate oil for general purpose domestic heating for use in burners not requiring No. 1 fuel oil (an oil intended for use in vaporizing pot-type burners) and having the following inspections:

|    |                                                  |              |
|----|--------------------------------------------------|--------------|
| 45 | Flash point, ° F. (min.)                         | 100 or legal |
| 45 | Pour point, ° F. (max.)                          | 20           |
|    | Water and sediment, vol. percent (max.)          | 0.10         |
|    | Carbon residue on 10% bottoms, percent (max.)    | 0.35         |
|    | Distillation temperature, ° F., 90% point (max.) | 675          |
| 50 | Viscosity, SUS, 100° F. (max.)                   | 40           |
| 50 | Viscosity, kinematic, cs., 100° (max.)           | 4.3          |
|    | Gravity, ° API (min.)                            | 26           |

The combustion improvement agent subjected to the foregoing test was the monohydrazinium salt of oil-soluble alkylbenzene sulfonic acids. The monohydrazinium sulfonate employed in the test was prepared by reacting hydrazine (95% hydrazine, 5% water) at room temperature in approximately equimolar proportions with a 47 percent solution in oil of oil-soluble alkylbenzene sulfonic acids having a combining weight (average molecular weight) of about 445, with the number of alkyl carbon atoms per molecule averaging about 20.5. The reaction mixture was cooled during addition of hydrazine to remove heat of reaction and to maintain the reaction mixture at about room temperature. The reaction product was diluted with hexane and filtered to remove insoluble matter, principally hydrazine sulfate. Hexane was then removed by evaporation on a steam bath. The resulting sulfonate comprised an approximately 50 percent solution in oil of monohydrazinium oil-soluble alkylbenzene sulfonate.

In order to demonstrate the extent of the improvement obtained with the test additive, test fuel A was also subjected to the test without addition of the combustion improvement agent.

In the following table there are tabulated the results obtained in the combustion tests described above.

The results of the tests are presented in Table C below:

Table A

| Composition                                                                      | Smoke Disc Number at— |                      |                    |                      |                     |                     |                     |                     |
|----------------------------------------------------------------------------------|-----------------------|----------------------|--------------------|----------------------|---------------------|---------------------|---------------------|---------------------|
|                                                                                  | 8% CO <sub>2</sub>    | 8.5% CO <sub>2</sub> | 9% CO <sub>2</sub> | 9.5% CO <sub>2</sub> | 10% CO <sub>2</sub> | 11% CO <sub>2</sub> | 12% CO <sub>2</sub> | Avg. Smoke Spot No. |
| 1. Test Fuel A-----                                                              | 6.20                  | 5.65                 | 5.05               | 4.45                 | 3.75                | 2.70                | 2.70                | 4.36                |
| 2. Test Fuel A plus 0.05 Wt. percent (active component) Hydrazine Sulfonate----- | 4.95                  | 4.10                 | 3.50               | 3.05                 | 2.65                | 2.15                | 2.00                | 3.20                |

The data presented in the foregoing table indicate that 20 a marked improvement in burning qualities of fuel oils is obtained by incorporation therein of the combustion improvement agents of this invention. Thus, 0.05 percent hydrazine sulfonate in test fuel A produced an average improvement of more than 26 percent in the smoke spot 25 number.

The addition agent and the test fuel described in the foregoing tests are illustrative only. Substitution of other sulfonates disclosed herein in the same or equivalent proportions in the foregoing test compositions will produce similar benefits. Examples of other fuel compositions included by this invention are shown in the following table.

Table B

35

| Base Oil                                                                       | Gravity, ° API | Aromatics, Percent | Addition Agent                                                        | Weight Percent Add. A |
|--------------------------------------------------------------------------------|----------------|--------------------|-----------------------------------------------------------------------|-----------------------|
| No. 2 Fuel Oil-----                                                            | 32.6           | 28.7               | Dihydrazinium p-C <sup>6</sup> H <sub>4</sub> Alkylbenzene Sulfonate. | 0.2                   |
| Do-----                                                                        | 32.6           | 28.7               | Monohydrazinium Mahogany Sulfonate. <sup>1</sup>                      | 0.1                   |
| No. 4 Fuel Oil (No. 6 Fuel Oil red. to 186.5 SUS/100° F. w. TCC Heavy Gas Oil) | 17.4           | 40+                | do. <sup>1</sup>                                                      | 0.1                   |

<sup>1</sup> Avg. M. W. of mahogany acid=435.

It is emphasized that the problem with which the present invention is concerned involves only fuel oils that are normally burned in fuel oil burners that utilize middle distillate and heavier oils and that normally exhibit severe smoking and soot forming tendencies in such usage. As indicated, such oils are those having an API gravity less than 34°. The problem with which this invention is concerned is especially serious in the case of distillate fuel oils of the type described because combustion quality is of primary consideration with such oils. Although a clean combustion problem also exists in the case of residual fuel oils suitable for use in atomizing type burners, the relatively low price of such fuels and the absence of a superior competitive fuel renders the problem less serious in the case of such oils.

In order to demonstrate the nature of the problem with which the present invention is concerned, a number of fuel oils having varying densities and aromatics contents were subjected to a combustion test substantially similar to that described above, but carried out in a Timken Vertical Rotary Wall Flame Burner, Model F, installed in a Weil-McLain Type 4-S-19 steam boiler, in order to determine the burning characteristics of the oils. These tests were carried out at 11.0% CO<sub>2</sub> in the flue gas, a recommended figure for the burner model in ques-

Table C

| Fuel Oil                                                           | Gravity, ° API | Percent Aromatics | Smoke Disc No. |
|--------------------------------------------------------------------|----------------|-------------------|----------------|
| 1. FCC No. 2 Distillate-----                                       | 25.8           | 42                | 4.4            |
| 2. 50/50 by Vol. Eastern Venezuela St. Run and FCC No. 2 Dist----- | 28.0           | 29.3              | 2.8            |
| 3. Fixed Bed Cat. Cracked No. 2 Dist-----                          | 29.0           | 28.7              | 3.0            |
| 4. TCC No. 2 Distillate-----                                       | 30.9           | 24.0              | 2.2            |
| 5. 80/20 by Vol. E.V.S.R. and FCC No. 2 Dist-----                  | 32.1           | 23.2              | 1.3            |
| 6. TCC Raffinate-----                                              | 34.5           | 16.3              | 0.6            |
| 7. 50/50 TCC Raffinate and West Tex as St. Run-----                | 35.6           | 15.6              | 0.6            |
| 8. Blend of Kerosene and Gas Oil, 50/50 by Vol-----                | 41.8           | 13.9              | 0.4            |
| 9. Kerosene-----                                                   | 42.6           | 14.0              | 0.7            |

From the results shown in the foregoing table, it will be seen that fuel oils having an API gravity of less than about 34° and an aromatics content of about 20 percent or more produce a relatively high smoke spot number which is a measure of the smoking and sooting tendencies of the oils. Even a small decrease in API gravity of such lower gravity oils normally results in a disproportionate increase in the smoke spot rating. In contrast, oils having a gravity above 34° API produced a low smoke spot number, and little difference in smoke spot number resulted among such oils despite substantial differences in API gravity.

The oil-soluble petroleum sulfonic acids whose salts are employed in the fuel oil compositions of this invention 50 are the sulfonic acids known as mahogany acids. These acids, together with water-soluble green acids, are produced during the acid refining of lubricating oil distillates. Methods of recovering these acids are well known and form no part of the invention.

If desired, the fuel oil compositions of this invention 55 may contain in addition to the compounds previously discussed oxidation inhibitors, corrosion inhibitors, anti-foam agents, ignition quality improvement agents, sludge inhibitors, color stabilizers and other addition agents adapted to improve the oils in one or more respects.

Obviously, many modifications and variations of the invention as herein described may be resorted to without departing from the spirit or scope thereof. Therefore, 60 only such limitations should be imposed as are indicated in the appended claims.

We claim:

1. A fuel oil composition comprising a major amount of a hydrocarbon fuel oil that has an API gravity less than about 34°, and that normally tends to form smoke 65 and soot during combustion, and containing a small amount, sufficient to reduce the smoke and soot forming tendencies of the oil, of a salt of hydrazine and an oil-soluble hydrocarbon sulfonic acid selected from the group 70 consisting of petroleum sulfonic acids and long-chain aliphatic hydrocarbon-substituted benzene sulfonic acids.

2. The composition of claim 1 where said fuel oil is a distillate fuel oil.
3. The composition of claim 1 where said small amount is about 0.02 to about 0.5 percent by weight of the composition.
4. The composition of claim 1 where said member is a salt of hydrazine and an oil-soluble, long-chain aliphatic hydrocarbon-substituted benzene sulfonic acid.
3. The composition of claim 1 where said member is a monohydrazinium salt of an oil-soluble alkylbenzene sulfonic acid containing 14 to 36 alkyl carbon atoms. 10
6. The composition of claim 1 where said member is a salt of hydrazine and oil-soluble petroleum sulfonic acids.
7. A salt of hydrazine and an oil-soluble, long-chain aliphatic hydrocarbon-substituted benzene sulfonic acid. 15
8. A salt of hydrazine and oil-soluble petroleum sulfonic acids.
9. A monohydrazinium salt of an oil-soluble alkylbenzene sulfonic acid containing 14 to 36 alkyl carbon atoms. 20
10. A fuel oil-soluble salt of hydrazine and an oil-

soluble hydrocarbon sulfonic acid selected from the group consisting of petroleum sulfonic acids and long-chain aliphatic hydrocarbon-substituted benzene sulfonic acids, said salt being capable of reducing the smoke and soot forming tendencies of hydrocarbon fuel oils.

References Cited in the file of this patent

UNITED STATES PATENTS

|           |               |               |
|-----------|---------------|---------------|
| 2,027,394 | McMullan      | Jan. 14, 1936 |
| 2,062,675 | Rather et al. | Dec. 1, 1936  |
| 2,270,681 | De Groote     | Jan. 20, 1942 |
| 2,321,496 | Liberthson    | June 8, 1943  |
| 2,650,198 | Kronig        | Aug. 25, 1953 |
| 2,660,562 | Axe et al.    | Nov. 24, 1953 |
| 2,702,819 | Axe et al.    | Feb. 22, 1955 |

OTHER REFERENCES

"The Chemistry of Hydrazine," by Audrieth, John Wiley and Sons Inc., 1951, pp. 224-232.

UNITED STATES PATENT OFFICE  
CERTIFICATION OF CORRECTION

Patent No. 2,971,827

February 14, 1961

Arthur V. Churchill et al.

It is hereby certified that error appears in the above numbered patent requiring correction and that the said Letters Patent should read as corrected below.

Column 1, line 18, for "improve" read -- improvement --; column 5, Table B, column 4, second line thereof, for "p-C<sup>24</sup>" read -- p-C<sub>24</sub> --; column 7, line 9, for "3. The composition" read -- 5. The composition --.

Signed and sealed this 20th day of June 1961.

(SEAL)

Attest:

ERNEST W. SWIDER

Attesting Officer

DAVID L. LADD

Commissioner of Patents